

## 1

3,243,291

### HIGH-TEMPERATURE ALLOY

Clayton D. Dickinson, Port Washington, and Sam Friedman, Great Neck, N.Y., assignors to General Telephone and Electronics Laboratories, Inc., a corporation of Delaware

No Drawing. Filed Oct. 29, 1963, Ser. No. 319,688  
4 Claims. (Cl. 75—176)

This invention relates to alloys for use at elevated temperatures and in particular to tungsten-base alloys containing additions of carbon and a reactive material.

Recent developments in aircraft and space vehicles have created a need for metals which have high strength at elevated temperatures yet remain ductile at relatively low temperatures. In addition, these metals must exhibit high recrystallization temperatures. Known materials are not satisfactory for many high temperature applications and it is therefore an object of our invention to provide alloys having the required characteristics.

In the present invention, tungsten-base alloys are provided which contain small additions of carbon and reactive metals selected from the group consisting of hafnium, zirconium and titanium. These ternary alloys contain between 0.004 and 0.05 percent carbon and between 0.01 and 2.0 percent reactive metal, the balance being tungsten. By varying the constituents within the specified ranges the best combination of mechanical properties and ease of fabricability may be obtained for a given application.

In particular, at a temperature of 1650° C., ultimate tensile strengths in the range 25,000 to 73,000 pounds per square inch are exhibited by the alloys as compared to

10

5

15

20

25

30

## 2

### EXAMPLE I

Elemental powders of carbon and tungsten were blended with hafnium hydride to form a uniform mixture which was then subjected to a pressure of approximately 50,000 pounds per square inch to form a billet. The billet was next sintered at about 2300° C. for approximately 90 minutes to mutually diffuse the different ingredients thereby forming a solid solution of hafnium in tungsten, the carbon being partitioned between tungsten carbide and a solid solution of carbon in tungsten. The billet was then fabricated by rolling initially at 1850° C.—1950° C. with final rolling at 1550° C. to form sheets having a thickness of approximately 0.040 inch. While a powder metallurgy process was used in forming the sheets, it shall be understood that the alloys may also be consolidated by other processes such as vacuum arc-casting. Fabrication may be accomplished by other techniques such as extruding, forging or drawing to produce the desired wrought form. Measurements of ultimate tensile strength, stress-rupture strength, recrystallization temperature and ductile-to-brittle transition temperature were carried out for a number of alloys.

The recrystallization temperature was established by determining at what temperature the fibrous structure of the wrought alloy completely disappeared and recrystallization was essentially complete. The ductile-to-brittle transition temperature was measured by bending a wrought sample over a radius four times the thickness of the sheet through a 105° angle at several temperatures and determining the minimum temperature at which deformation occurred without cracking. Characteristics of wrought tungsten-hafnium-carbon alloys of different compositions are shown in Table I.

Table I

| Alloy, percent by weight |       |       | Ultimate tens. strength at 1,650° C. (p.s.i.) | Stress-rupt. in 10 hours at 1,650° C. (p.s.i.) | Recryst. temp. (° C.) | Ductile-to-brittle trans. temperature (° C.) |
|--------------------------|-------|-------|-----------------------------------------------|------------------------------------------------|-----------------------|----------------------------------------------|
| Hf                       | C     | W     |                                               |                                                |                       |                                              |
| 0.01                     | 0.013 | Bal.  | 25,000                                        | -----                                          | 1,700                 | 150-175                                      |
| 0.03                     | 0.017 | ----- | 61,700                                        | -----                                          | 1,900                 | -----                                        |
| 0.24                     | 0.004 | ----- | 73,800                                        | -----                                          | 1,800                 | ≤125                                         |
| 0.53                     | 0.033 | ----- | 67,800                                        | -----                                          | -----                 | 150-175                                      |
| 0.48                     | 0.037 | ----- | 66,200                                        | 30,000                                         | -----                 | ≥175                                         |
| 0.49                     | 0.050 | ----- | 61,500                                        | -----                                          | 1,850                 | 150                                          |
| 1.07                     | 0.015 | ----- | 68,500                                        | -----                                          | -----                 | -----                                        |
| 2.0                      | 0.015 | ----- | 58,000                                        | -----                                          | -----                 | -----                                        |

15,000 pounds per square inch for unalloyed tungsten. The temperature above which the alloy becomes substantially ductile (the brittle-to-ductile transition temperature) is equal to or less than that for unalloyed tungsten. The high strengths and high recrystallization temperatures obtained in the tungsten-reactive metal-carbon alloys are due to the formation, during fabrication, of a uniformly dispersed reactive metal carbide having particle sizes predominantly in the range 200 to 1000 Angstroms. The improved properties are the result of both the chemical constituents and the state of aggregation of these constituents. Transportation of the reactive metal is believed to occur during fabrication to produce particles dispersed throughout the matrix, the diameter of these particles being in the range 200 to 1000 Angstroms.

60

By contrast, the following values are reported for unalloyed tungsten:

Ultimate tensile strength at 1650° C. ----- 15,00 pounds per square inch.  
Recrystallization temperature ----- 1600° C.  
Ductile-to-brittle transition temperature ----- 200 °C.

70

Carbon base alloys containing 0.15 to 1.0 hafnium and 0.015 to 0.035 carbon exhibit an optimum combination of ultimate tensile strength, recrystallization temperature, ductile-to-brittle transition temperature and fabricability.

**3**  
**EXAMPLE II**

An alloy consisting of tungsten, zirconium, and carbon was prepared by the method described for the alloy of Example I. Table II gives the characteristics of various compositions of this alloy.

*Table II*

| Alloy, percent by weight |       |       | Ultimate tens. strength at 1,650° C. (p.s.i.) | Recrystall. temperature (° C.) | Ductile-to-brittle transition temp. (° C.) |
|--------------------------|-------|-------|-----------------------------------------------|--------------------------------|--------------------------------------------|
| Zr                       | C     | W     |                                               |                                |                                            |
| 0.01                     | 0.015 | Bal.  | 35,000                                        | -----                          | -----                                      |
| 0.03                     | 0.018 | ----- | 70,800                                        | 1,700                          | 125-150                                    |
| 0.11                     | 0.012 | ----- | 62,400                                        | >1,850                         | ≤125                                       |
| 0.11                     | 0.050 | ----- | -----                                         | 1,725                          | -----                                      |
| 0.13                     | 0.004 | ----- | 61,100                                        | 1,825                          | 125-150                                    |
| 0.45                     | 0.036 | ----- | 69,600                                        | 1,800                          | 125-150                                    |
| 0.015                    | 0.015 | ----- | 64,000                                        | -----                          | -----                                      |

Carbon base alloys containing 0.05 to 0.5 percent zirconium and 0.01 to 0.025 percent carbon exhibit a highly desirable combination of ultimate tensile strength, recrystallization temperature, ductile-to-brittle transition temperature and fabricability.

**EXAMPLE III**

An alloy consisting of 0.24 percent titanium, 0.027 percent carbon with the balance tungsten was prepared by the method of Example I. This alloy has the following characteristics:

*Table III*

Ultimate tensile strength ----- 58,700 p.s.i.  
Recrystallization temperature ----- 1900° C.  
Ductile-to-brittle transition  
temperature ----- Between 125  
and 150° C.

From these results it is apparent that our alloys exhibit high strength at elevated temperatures and are ductile at low temperatures. The alloys also have high recrystallization temperatures as compared to unalloyed tungsten. For applications where a high melting point is desired, the composition containing the minimum alloying ingredients

consistent with desired mechanical properties have been found most suitable.

As many changes could be made in the above described processes it is intended that all matter contained therein shall be interpreted as illustrative and not in a limiting sense.

**4**

What is claimed is:

1. A tungsten-base alloy consisting essentially of between 0.004 and 0.05 percent carbon and between 0.01 and 0.45 percent zirconium, the balance being tungsten.

2. A tungsten-base alloy consisting essentially of between 0.01 and 0.025 percent carbon and between 0.05 and 0.45 percent zirconium, the balance being tungsten.

3. A tungsten-base alloy consisting essentially of approximately 0.027 percent carbon and approximately 0.24 percent titanium, the balance being tungsten.

4. A tungsten-base alloy consisting essentially of between 0.004 and 0.05 percent carbon and between 0.01 and 0.45 percent zirconium, the balance being tungsten, said alloy having uniformly dispersed zirconium carbide particles distributed therein, the size of said particles being predominantly in the range 200 to 1000 Angstroms.

35

**References Cited by the Examiner**

**UNITED STATES PATENTS**

3,113,863 12/1963 Chang ----- 75-174  
3,116,145 12/1963 Semchyshen ----- 75-176  
3,169,860 2/1965 Semchyshen ----- 75-176

DAVID L. RECK, *Primary Examiner.*

C. N. LOVELL, W. C. TOWNSEND,

*Assistant Examiners.*

45